

## UNITED STATES PATENT OFFICE.

OSKAR KALTWASSER AND LEOPOLD KIRBERGER, OF BERLIN AND BERLIN-CHARLOTTENBURG, GERMANY, ASSIGNORS TO ACTIEN GESELLSCHAFT FÜR ANILIN FABRIKATION, OF BERLIN, GERMANY.

### PROCESS FOR DYEING SKINS, HAIRS, AND THE LIKE.

No Drawing.

Application filed January 25, 1922. Serial No. 531,778.

*To all whom it may concern:*

Be it known that we, OSKAR KALTWASSER and LEOPOLD KIRBERGER, citizens of the German Republic, residing at Berlin, Germany, and Berlin-Charlottenburg, Germany, our P. O. address being Urbanstr. 178, Berlin, Germany, and Schillerstr. 121, Berlin, Germany, have invented certain new and useful Improvements in Processes for Dyeing Skins, Hairs, and the like, of which the following is a specification.

Our invention relates to a new process for dyeing skins, hairs and the like and consists in acting with a solution of 2,7-dioxynaphthalene in the presence of an oxidizing agent upon mordanted or non-mordanted material.

The tints thus obtained are generally speaking gray inclining to green of a very good fastness.

20 The following example illustrates our invention without limiting it:

The well-washed skin is handled for some hours at ordinary temperature in a bath which contains per liter 2 grams 2,7-dioxynaphthalene and 30 grams of hydrogen peroxide (about 3% strength). The skin is then well washed and finished as usual, a gray shade being obtained.

The tints obtained on skins prepared with

chromium mordants are brownish gray, 30 those on skins prepared with copper mordants are greenish gray; on skins prepared with iron mordants a gray is produced.

By dyeing in an alkaline solution, for example by addition of 2 grams of ammonia 35 (of 25% strength) to the above dyeing bath dyeings which are more yellowish result.

Having now described our invention and the manner in which it may be performed what we claim is,—

1. The herein-described process for dyeing furs, feathers, hairs and the like material, consisting in acting on the material to be dyed with a solution of 2,7-dioxynaphthalene in the presence of an oxidizing 45 agent.

2. The herein-described process for dyeing furs, feathers and the like material, consisting in acting on the mordanted material with a solution of 2,7-dioxynaphthalene in 50 the presence of an oxidizing agent.

In testimony whereof we affix our signatures in presence of two witnesses.

OSKAR KALTWASSER.  
LEOPOLD KIRBERGER.

Witnesses:

C. HOLTZERMANN,  
CHARLES L. TURRILL.